

## UNITED STATES PATENT OFFICE

2,122,418

PRODUCT AND PROCESS OF PREPARING  
SAME

Ernest K. Gladding, Buffalo, N. Y., and Dorothy Bateman Maney, Old Hickory, Tenn., assignors, by mesne assignments, to E. I. du Pont de Nemours & Company, Wilmington, Del., a corporation of Delaware

No Drawing. Application June 17, 1936,  
Serial No. 85,768

22 Claims. (Cl. 91—68)

This invention relates to coated sheets or films and it particularly pertains to regenerated cellulose film coated with a moistureproofing composition which tenaciously adheres to or is anchored to the base film even when in direct contact with water for prolonged periods of time or when used as a wrapping tissue directly in contact with products containing large amounts of water or moisture. The invention also pertains to methods for producing such coated sheets or films.

This application is a continuation in part of the application of Ernest K. Gladding and Dorothy E. Bateman, Ser. No. 731,603, filed June 21, 1934 for "Product and process of preparing same."

Ordinary sheets or films of regenerated cellulose have been rendered moistureproof by coating with a moistureproofing composition comprising in its preferred form a flowable solution of a cellulose derivative, a wax or wax-like material, a blending agent and a plasticizer. These coated sheets or films are very effective as a wrapping material for such products as bread, cake, candy, or the like which it is desired to maintain in substantially their original fresh condition without any change in moisture content. Such coated sheets or films, when used as a wrapping material which is directly held in contact with products having an exceedingly high water or moisture content, such as butter, cheese, wet or frozen fish, ice cream or the like, and when such articles are kept over long periods of time in storage, have the disadvantage that the moistureproof coating tends to loosen and/or flake off from the sheet of regenerated cellulose and to thereby lessen the moistureproof quality of the wrapping material.

It is an object of this invention to provide a flexible, substantially odorless, non-fibrous cellulosic sheet or film having a surface coating which will adhere tenaciously to the cellulosic sheet or film. A further object comprises the production of films of this character having a moistureproofing coating comprising a cellulose derivative, a wax or wax-like material, a blending agent and a plasticizer. A still further object of the invention comprises a simple, workable process, directly applicable to existing equipment, such as is used for the manufacture of regenerated cellulose sheets or films, for producing products having the characteristics described.

A further object of the invention resides in the production of transparent, flexible, non-fibrous, cellulosic sheets or films prepared by precipitation from an aqueous cellulosic dispersion, coated and/or sized with an amino polymer, and having

a moistureproof surface coating which remains firmly anchored to the cellulosic sheet or film even when in direct contact with water over long periods of time.

A specific object of the invention resides in the production of transparent, flexible, substantially odorless, non-fibrous cellulosic sheets or films prepared by precipitation from an aqueous cellulosic dispersion, coated and/or sized with a de-acetylated chitin, and having a moistureproof surface coating which remains firmly anchored to the cellulosic sheet or film even when in direct contact with water or moisture over a prolonged period of time.

Other objects of the invention will appear from the following description.

These objects are accomplished by the following invention which, in its preferred form, contemplates forming a cellulosic sheet or film, applying to said sheet or film a surface coating having moistureproofing characteristics and applying directly to the cellulosic base and intermediate said base and the surface coating, a coating and/or sizing of an amino polymer and preferably of a de-acetylated chitin.

The following examples illustrate modes of applying the principles of the invention.

## Example I

A sheet of regenerated cellulose in the gel state, which has been cast from viscose, desulfured, bleached, and washed free from impurities in the usual manner on the casting machine and is ready for the glycerin treatment, is led through an aqueous glycerin bath, which, in addition to 4 1/2 per cent by weight of glycerin, also contains one per cent by weight of a de-acetylated chitin, and 0.28 per cent by weight of acetic acid (calculated as 100 per cent acetic acid).

Acetic acid is used in order to render the de-acetylated chitin soluble. In this example, the acetic acid used corresponds to 75 per cent of the amount of acid theoretically required to completely react with the de-acetylated chitin used when a ratio of 161 to 60 is employed to express the relation of de-acetylated chitin to acetic acid in terms of molecular weights.

The sheet of regenerated cellulose is held in contact with the aqueous solution of the salt of de-acetylated chitin and glycerin for from 10 to 20 seconds after which the excess solution is removed from the sheet by means of squeeze rolls which reduce the water content of the sheet to between three and four times the weight of the cellulose, after which the sheet of regenerated

cellulose, wet with the solution, is ready to be dried. During the drying of the sheet, the acetate of de-acetylated chitin becomes converted into the de-acetylated chitin and acetic acid, the volatile acetic acid being removed in the drying air and the sheet of regenerated cellulose being left with a transparent coating or sizing of de-acetylated chitin which is insoluble in both water and organic liquids.

10 The drying of the sheet of regenerated cellulose which has been treated with the aqueous glycerin solution containing the size (the de-acetylated chitin) may be carried out according to the usual method for drying regenerated cellulose sheeting 15 on the casting machine by bringing the sheet directly from the squeeze rolls into contact with heated rolls which dry the sheet at temperatures preferably between 50 and 90 degrees centigrade. However, there may be a tendency for 20 the size to be deposited on the dryer rolls when they become wet with the solubilized de-acetylated chitin from the wet film passing over them. This deposit, resulting from the heat acting on the soluble size, may flake off from time to time 25 on the fresh film passing over the dryer rolls, thereby imparting a faintly mottled appearance to the finished film.

Therefore, in this preferred example, the regenerated cellulose sheet, wet with a solution of 30 glycerin and the size, after passing through the squeeze rolls and before coming into contact with the dryer rolls, is first given a preliminary partial drying out of contact with any surface by passing the sheet through air heated to an 35 elevated temperature by means of any suitable arrangement, whereby the moisture content of the sheet is reduced to any desired extent, for instance, from one-tenth to one-half of its initial water content before coming in contact with 40 the dryer rolls of the casting machine to complete the drying operation in the usual manner.

The resulting sheet of regenerated cellulose coated or sized with an insoluble deposit of de-acetylated chitin may be conditioned if necessary to bring it to the desired moisture content 45 and is then coated with a moistureproofing composition of the following formula:

| Parts by weight          |       |
|--------------------------|-------|
| 50 Pyroxylin             | 6.75  |
| Gum damar                | 1.64  |
| Dibutyl phthalate        | 2.80  |
| Paraffin, M.P. 60-61° C. | 0.48  |
| Zinc stearate            | 0.15  |
| 55 Ethyl acetate         | 56.34 |
| Toluene                  | 28.53 |
| Alcohol                  | 3.20  |
| Acetone                  | 0.11  |

60 The sheet is passed through the moistureproofing composition, the excess of which is removed by scraping or any suitable means, and the coated sheet is dried at a temperature above the melting point of the wax, after which the finished sheet may be conditioned if necessary to bring it to the 65 desired moisture content. The resulting product is a sheet of regenerated cellulose with a moistureproofing coating, which is substantially odorless, transparent, flexible, and moistureproof, and to which, by virtue of the sheet being coated 70 or sized with a de-acetylated chitin, the moistureproof coating adheres or is anchored very tenaciously when the sheet is in direct contact with water or is used as a wrapping directly in contact with products containing large amounts 75 of water or moisture such as butter, cheese, wet

or frozen fish, ice cream, or the like, for very substantial periods of time, for example, for a month or more.

#### Example II

5 A sheet of regenerated cellulose in the gel state is passed through an aqueous bath containing 4½ per cent by weight of glycerin, 0.7 per cent by weight of a de-acetylated chitin, and 0.2 per cent by weight of 85% formic acid, or any other 10 amount of formic acid sufficient to render the size water-soluble.

In this example, the amount of formic acid used is 80% of that theoretically required to completely react with the de-acetylated chitin to 15 form the desired formate, assuming the molecular ratio of de-acetylated chitin to formic acid to be 161 to 46.

20 After being held in contact with this bath for 10 to 20 seconds, the cellulosic sheet is freed from excess solution by means of squeeze rolls so that the water content of the sheet is between three and four times the weight of the cellulose and the sheet is then dried either by being led directly over heated rolls, or as in Example I, by means of a preliminary partial drying in hot air out of 25 contact with any surface, followed by passage over dryer rolls to complete the drying. In either case the drying of the sheet may be accompanied by a treatment with gaseous ammonia which 30 facilitates the conversion of the water-soluble formate salt of the de-acetylated chitin to an insoluble product.

A moistureproofing coating is applied to the 35 sheet of regenerated cellulose treated as described above in this example by passing the sheet through a bath comprising ethyl cellulose, a wax, a blending agent and a plasticizer, removing the excess moistureproofing bath and removing the solvent at a temperature above the 40 melting point of the wax, after which the coated sheet is brought to the desired moisture content. The resulting product exhibits the same properties which have been described for the moisture-proof film produced in accordance with Example 45 I.

#### Example III

A finished or dry sheet of glycol cellulose is 50 passed through an aqueous solution containing 0.5% by weight of de-acetylated chitin which has been converted to the acetate by acetic acid in an amount which is 0.15% by weight of the aqueous solution (calculated on the basis of 100% acetic acid). After removing the excess solution 55 from the sheet in any suitable manner, the sheet is dried at 80 degrees centigrade and subsequently coated with a moistureproofing composition comprising a solution of nitrocellulose, gum damar, paraffin and dibutyl phthalate. The excess moistureproofing material and the solvent 60 may be removed as described in the preceding example.

#### Example IV

The diethylaminoethyl methacrylate polymer 65 produced in accordance with the procedure outlined in Example B (below) is dissolved in dilute acetic acid containing 5-6% glycerol to form a solution containing 0.25-1.00% of the resinous polymer, sufficient acetic acid being used to just 70 solubilize the polymer. Sheets of gel regenerated cellulose film are immersed in this solution and allowed to remain five minutes, whereupon they are removed and the excess solution drained off. The sheets are then dried in an oven at 120° C. 75

for about 10 minutes, after which they are coated with a moistureproofing lacquer as in Example I to produce a clear, transparent, flexible and moistureproof film. These coated films show an anchorage only slightly inferior to that obtained with the use of deacetylated chitin as the anchoring agent.

*Example V*

Sufficient beta-amino ethoxyethyl cellulose to form a 2% solution is dissolved in an aqueous mixture containing 1.5% acetic acid and 5% glycerol. Sheets of gel regenerated cellulose film freed from excess water are immersed in this solution at room temperature for 5 minutes, after which they are removed and allowed to drain, the excess of the rather viscous solution being scraped off by means of glass rods. The treated film is then placed on a drying frame and dried in an oven at 120° C. for 10 minutes. The dry film is then coated with a moistureproofing lacquer in the usual manner to produce a clear, transparent, flexible and moistureproof product. The anchorage of the moistureproofing coating is equal to or better than that obtained through the use of deacetylated chitin as the anchoring agent.

*Example VI*

An aqueous solution containing 2% of diethyl-amino methyl zein is prepared by dissolving the amino polymer in dilute acetic acid containing 0.28 parts of acetic acid for each part of the zein derivative and 5-6% glycerol. Films of gel regenerated cellulose are treated as in the preceding examples, the drying time being 30 minutes at 120° C. The anchorage obtained after moistureproofing is somewhat inferior to that obtained through the use of de-acetylated chitin alone. The use of a 1% solution of the zein derivative results in some improvement in the anchorage and the use of a combination of 1% solution of the zein derivative and 1% solution of deacetylated chitin produces anchorage results which are better than those obtained with either when used alone in 2% concentration.

*Example VII*

An aqueous solution containing 2% piperidyl methyl zein is prepared by dissolving in water containing 0.28 part of acetic acid per part of zein derivative and 5-6% glycerol. Gel regenerated cellulose film treated with this solution and dried for 30 minutes at 120° C. as described above and coated with a moistureproofing composition shows an improved anchorage which, though inferior to that of de-acetylated chitin is quite satisfactory.

*Example VIII*

A 2% solution of the phenol-formaldehyde-dimethylamine resin (Example E below) is prepared by dissolving the resin in an aqueous solution containing 1.5% acetic acid and 6% glycerin and this solution was used as a treating bath for regenerated cellulose film. The treated film is dried for 30 minutes at 120° C. and the moistureproof product shows anchorage approximately equal to that of de-acetylated chitin with some improvement over the latter when the anchorage tests were made in water containing 0.1% acetic acid.

*Example IX*

A meta-cresol-dimethylamine-formaldehyde resin similar to the resin described in Example E (below) is dissolved in dilute acetic acid con-

taining 5-6% glycerol to form a solution containing 2% of the resin. When used as the anchoring agent, as in the preceding examples, the results obtained are comparable to those obtained with deacetylated chitin. A 1% solution of the resin appears to be substantially equally satisfactory and the use of a solution containing 1% of this resin and 1% of de-acetylated chitin results in an anchorage which is somewhat better than that obtained with either of these ingredients when used alone in 2% concentration.

*Example X*

A dicyclohexyl amino ethyl methacrylate prepared in a manner similar to that described in Example B (below) may be used in either its monomeric or polymeric forms. Mixtures of the monomer and polymer have been found to be particularly useful, the resinous material being brought into solution by means of dilute acetic acid. A 2% solution is capable of producing a final material which will show an anchorage approximately equal to that of the de-acetylated chitin. The anchorage can be improved somewhat by using as the anchoring agent a combination of these monomers and/or polymers with de-acetylated chitin.

This invention contemplates, as a base, any smooth, dense, non-porous, non-fibrous cellulosic sheet or film which may be precipitated from an aqueous cellulosic dispersion. Thus, the scope of the invention includes the use of sheets or films of regenerated cellulose, whether precipitated from solutions of viscose, cuprammonium cellulose, or any other aqueous solution or dispersion of cellulose, and it also contemplates the use of sheets or films of such cellulose esters and ethers as are precipitated from aqueous solutions or dispersions, such as glycol cellulose, cellulose glycolic acid, methyl cellulose and ethyl cellulose of low alkyl content, cellulose phthalate, and other cellulose products similar to those described. When any given coating composition is applied to such cellulosic sheets or films, the coating composition will not penetrate therethrough and will normally result in a surface coating. It is desired to emphasize the fact that the preferred form of the invention is directed to the treatment of regenerated cellulose sheets or films since it is in this form that the invention may be applied with the greatest advantages.

As a surface coating, the invention contemplates the use of any coating composition containing a cellulose derivative base, such as cellulose nitrate, cellulose acetate, ethyl cellulose, benzyl cellulose or the like, which may be modified as desired by the addition of blending agents, waxes, plasticizers, et cetera. In its preferred form, this invention contemplates as a surface coating a moistureproofing coating comprising a cellulose derivative, a wax or wax-like material or other moistureproofing agent, a blending agent and a plasticizer. Such moistureproofing compositions are disclosed in Charch and Prindle U. S. Patent No. 1,737,187, issued November 26, 1929.

The invention also contemplates the anchoring to a cellulosic base of moistureproofing coatings which may not contain cellulosic material, e. g., rubber-wax or resin-wax coatings, and includes also the anchoring of coatings which may conceivably be used for purposes other than moistureproofing.

The amino polymers which are contemplated as coming within the scope of this invention are all

substantially insoluble in water and in 5% aqueous ammonia, but soluble in 2% aqueous acetic acid. The amino nitrogen may be primary, secondary or tertiary, part of an open chain or of a cyclic molecular structure.

6 The amino polymers which may be used as anchoring agents, as illustrated in the above examples, may be subdivided into several groups as follows:

10 1. The first group, closely related to though nevertheless distinct from cellulose, may be considered as hexose amine polymers, or more broadly as carbohydrate amine polymers, which have, where necessary, been purified and converted into 15 the acid soluble type. With or without such treatments, the highly polymeric molecule is built up by nature, and the amine nitrogen, as a rule, is present in the natural product. Those in which the nitrogen is present in the substance as 20 it exists naturally may be of marine or insect origin on the one hand, or vegetable origin on the other. De-acetylated chitin, which is by far the best example of a hexose amine polymer is, for example, of marine origin, and the polymers 25 obtained from fungi such as *aspergillus niger* are of vegetable origin. Examples of carbohydrate amine polymers in which the highly polymeric molecule has been built up by nature, but into which the amine nitrogen has been introduced 30 synthetically are the alkylamino celluloses. Regardless of the source of the nitrogen, this first group also includes various reaction products and chemical derivatives of carbohydrate amine polymers, provided of course that they have the 35 required solubility characteristics.

2. The second group of amino polymers comprises that group of synthetic resins, in the making of which ammonia in some instances and monomeric amino nitrogen containing bodies in 40 others have been employed. This group is distinct in that the highly polymeric molecules are built up wholly by artificial means, i. e., they are not synthesized by nature. The resins of this group may be considered broadly as those which contain 45 amino nitrogen and have the requisite solubility characteristics. The following types of resins are illustrative of the classes among which highly polymeric amino nitrogen containing bodies falling in this classification may be found. (a) 50 Resinous polymeric amino alcohol esters of acrylic acid and of its homologues substituted in the alpha position by a hydrocarbon radical, and (b) resinous reaction products of phenols, aldehydes and ammonia or primary or secondary amines.

55 (a) Examples of the first of the above subclasses of resins are beta-diethylaminoethyl alpha-methacrylate, beta-piperidyl-N-ethyl-alpha-methacrylate, and beta-dicyclohexyl aminoethyl alpha-methacrylate. These resins 60 may be prepared by spontaneous polymerization of the monomeric compounds, but for the purposes of the present invention, advantage can be taken of a unique property of the monomers, namely their ability to form polymerizable salts 65 with aqueous acids. The monomer as prepared may simply be dissolved in the stoichiometrical amount or more of aqueous acid and the solution heated with a polymerization catalyst such as benzoyl peroxide until polymerization of the salt 70 is effected.

(b) An example of the second of the above subclasses of resins having amino nitrogen and the specified solubilities is the reaction product of meta-cresol, formaldehyde and dimethyl- 75 amine. Other phenols such as phenol itself or

p-tertiary amyl phenol may be substituted for the cresol, and the ammonia or various primary or secondary amines for the dimethylamine. It is desirable in most cases, possible in all cases, and necessary in some cases, to react the amine or 5 ammonia with a part of the formaldehyde before adding the remainder. These resins are to be sharply distinguished from the phenol-aldehyde resins prepared in the presence of only catalytic amounts of ammonia or amines, which resins 10 cannot be employed in accordance with the methods of this invention because they lack the preponderance of amino nitrogen which induces the proper solubility characteristics. The molal ratio of amine to phenol which is used in making 15 the resins with which the present invention is concerned is on the order of 1:2.

3. The third group of amino nitrogen containing polymers included in this invention consists of protein derivatives containing sufficient amino 20 nitrogen to make them comply with our solubility requirements. Examples are piperidyl-methyl zein, dimethylaminomethyl zein, and diethylaminomethyl zein. These products may be made in one way as follows. The zein is first 25 suspended in water or dissolved in about 75% alcohol, preferably the latter. To the alcohol solution is added aqueous formaldehyde, a secondary amine and sufficient alcohol to keep the concentration at about the original figure. The mixture 30 is allowed to stand or may be heated gently until it becomes soluble in acetic acid, 6-18 hours, depending on temperature, usually being required. The final product, in order to be acid soluble, should have at least 8-10% basic amino nitrogen. 35 The maximum obtainable is around 22% and the products having the high percentages are the most desirable for use in the present invention.

40 Examples I to III are directed to the use of a de-acetylated chitin as an anchoring agent for the moistureproofing coating. Chitin is an acetylated carbohydrate amine polymer, and may be, for convenience, termed "chitose amine polymer", and after the removal of the acetate, as by saponification, the product, which is believed to be 45 a carbohydrate amine polymer, is capable of reacting with acids to form salts. The de-acetylated chitin referred to in the examples given above, may be prepared as described in the Rigby U. S. Pat. No. 2,040,879, issued May 19, 1936, one 50 method of preparation being described as follows:

#### Example 4

55 Shrimp, lobster or crab shells are treated first with a 1% solution of soda ash at boiling temperature for about six hours, after which the liquor is drained off and the shells washed with water until free of alkali as tested by phenolphthalein. The washed shells are then subjected 60 for a period of time to treatment with a 5% hydrochloric acid solution until all lime salts have been removed (10 to 12 hours at ordinary temperatures). After washing with water to remove the acid, the shells are given a second treatment with a 1% soda ash solution containing about 0.02% ordinary soap, the treatment being carried out at the boiling temperature of the solution for a period of about 8 hours. After this treatment the shells are drained free of the liquor 65 and water-washed until free of alkali as tested by phenolphthalein, whereupon they are centrifuged to remove as much water as possible. The shells are then treated with 40% sodium hydroxide at 70 110 degrees centigrade for about four hours, after 75

which they are again water-washed until free of alkali as tested by phenolphthalein. The residue is de-acetylated chitin, is pure white and, after drying at 65 degrees centigrade, may be used to prepare solutions in acids as desired.

The chitin may be partially or completely de-acetylated depending on the conditions present during the de-acetylation. The more complete the de-acetylation, the more soluble is the salt produced by reacting with acid. Thus chitose amine polymer, from which the acetyl substituent has been completely removed, forms the most soluble salt. However, during de-acetylation, some degradation of this chitose amine polymer takes place and the extent of degradation increases as the de-acetylation becomes more complete. Thus, for purposes of expediency, there must be a balance established between the completeness of de-acetylation and the degradation of the de-acetylated product. For ordinary purposes, it will be sufficient to use a product prepared from chitin which has been 85 to 90 per cent de-acetylated. It will be understood that this range of de-acetylation is not limitative since chitin, which has been de-acetylated to an extent as low as 50 per cent or lower or as high as 100 per cent, may be used with advantage.

It has been stated that chitin is believed to be an acetylated carbohydrate amine polymer. This is in accordance with the evidence presented in the literature. It is also believed to be an acetylated mixed or cross or inter-polymer of two carbohydrate amines. We do not wish, however, to be limited to theory, but cover the use 35 of the de-acetylated chitin regardless of its ultimate molecular composition.

While the de-acetylated chitin is the preferred form of anchoring agent for the coating which is used for the cellulose film, the invention also 40 contemplates the use of other carbohydrate amine polymers such as chondrosin which may be obtained by the de-acetylation of chondroitin (believed to be an acetylated carbohydrate 45 (chondrose) amine polymer and which is obtainable from animal cartilage in a manner similar to the preparation of chitin). Chondrosin may be solubilized with acids, e. g., acetic acid, and the product subsequently insolubilized in the same manner as described herein for the 50 treatment of de-acetylated chitin.

The carbohydrate amine polymer itself, termed herein a "de-acetylated chitin", is very insoluble in water, and in organic solvents, but it may be made soluble by causing it to react with any one of 55 a larger number of acids including acetic, formic, citric, glycolic, malic, maleic, succinic, adipic, phthalic, tartaric, benzoic and hydrochloric acids, and the like. Coatings or films prepared from aqueous solutions of these water-soluble salts, 60 upon being dried, preferably at an elevated temperature, are more or less rapidly rendered insoluble both in water and in organic solvents. In the case of salts formed by reacting with volatile acids, particularly volatile acids which 65 are only slightly ionized, like acetic acid, the conversion to insolubility is easily and quickly accomplished since the acid, being weak or slightly ionized is readily dissociated from its salt and being volatile is easily removed by heat, 70 leaving an insoluble residue. Salts formed from the non-volatile acids and/or from the highly ionized acids are much less readily converted to insolubility, and consequently in the practice of this invention, it is preferred to use salts of 75 the de-acetylated chitin and of volatile acids of

low ionization, of which acetic acid is an example. However, in the case of the salts formed from the non-volatile and/or highly ionized acids, these salts may be converted into the insoluble form by treatment with ammonia, as, for 5 example, in the form of gaseous ammonia (see Example II).

Any suitable concentration of de-acetylated chitin may be employed in the aqueous solution of its salt, depending upon the method of operation used and the amount of size which it is desired to have present in the finished cellulosic sheet. In general, it is preferred to use solutions in which the concentration of the de-acetylated chitin salt is equivalent to between 0.2 and 2.0 10 per cent by weight. As has been stated, however, higher or lower concentrations may be desirable at times for different effects or with different methods of applying the size. The amount of size present in the finished celulosic 15 sheet is controlled by the concentration of de-acetylated chitin salt in the solution and by the amount of this solution removed from the wet sheet by squeeze rolls or by other means, prior to the drying of the sheet. In the preferred form 20 of this invention, this amount ranges from 0.5 to 4.0 per cent of the weight of the sheet, although it may at times be desirable for certain purposes to have present in the sheet an amount of size greater or less than those included within 25 30 these limits.

The preparation of various amino polymers is fully discussed in Rigby U. S. Patent No. 2,040,-879, issued May 19, 1936, relating to the preparation of de-acetylated chitin; and in a number 35 of copending applications such as for instance, Graves Serial No. 21,807, filed May 16, 1935 relating to polymeric amino alcohol esters of alpha substituted acrylic acid; Harmon Serial No. 21,-810, filed May 16, 1935, relating to polymeric salts 40 of amino alcoholic esters of alpha substituted acrylic acid; Meigs Serial No. 59,643, filed January 17, 1936, relating to amino proteins; Hardy Serial No. 61,842, filed January 31, 1936, relating to amino celluloses soluble in dilute acetic acid; 45 Haskins Serial No. 61,806, filed January 31, 1936, relating to alkyl amino celluloses soluble in at least a stoichiometrical amount of 5% aqueous acetic acid; Balthis Serial No. 69,725, filed Mar. 19, 1936, relating to the resin prepared by reacting 50 vinyl ketone polymers such as methyl vinyl ketones with ammonia or a primary amine; Greenewalt Serial No. 69,723, filed Mar. 19, 1936, relating to hydrogenating ketone resins in the presence of ammonia or a primary or secondary 55 amine; and Harmon & Meigs Serial No. 85,820, filed June 17, 1936, relating to the preparation of amine-phenol-aldehyde resins.

To further illustrate the preparation of a few of these amino polymers the following examples 60 are given.

#### Example B

This compound is made by dissolving 117 grams (1 mol.) of beta-diethylaminoethanol and 400 65 grams (4 mols) of methyl methacrylate in 300 grams dry benzene containing 30 grams p-phenylene diamine, and heated in an oil bath under a 48" fractionating column fitted with a distilling head arranged for controlled reflux and 70 distilled until all the moisture present in the reagent has been removed. Beta-diethylaminoethyl methacrylate is isolated by collecting the fraction boiling at  $85 \pm 5^\circ$  C. at 5 mm. pressure, carefully washing 8 times with cold water to re- 75

move traces of p-phenylene diamine, drying with anhydrous magnesium sulfate, filtering, washing the drying agent with ether, combining the washings with the bulk of the product and then distilling the ether under reduced pressure in an atmosphere of nitrogen. The monomeric ester is left in the distilling glass as an almost colorless liquid which polymerizes spontaneously to a tough, transparent, pale amber polymer. When allowed to stand at room temperature or even at a lower temperature, the polymer was insoluble in water and in the common oxygenated organic solvents, soluble in acetone.

*Example C*

To a solution of 220 ccs. of formalin (37% aqueous formaldehyde) containing 1 gram of potassium carbonate, there is added 250 ccs. piperidene while the mixture is cooled with tap water. This methylolpiperidene solution is then added to a mixture of 1,500 ccs. of methanol, 75 ccs. of water, and 250 grams of zein. The solution is mixed thoroughly with mechanical agitation and allowed to stand over night. It is then centrifuged to remove insoluble materials and then concentrated in vacuo. The concentrated solution is poured into a large volume of water which results in the precipitation of the reaction product, which is washed several times by decantation and then finally pressed out and dried as rapidly as possible through the aid of a hot air blast in an oven at 50° C. The material is ground to a fine powder as soon as it is dry, the yield of piperidyl methyl zein being 239 grams. This material is readily soluble in dilute aqueous acetic acid, but insoluble in water or dilute ammonia solutions.

*Example D*

Fifty grams of polymeric methyl vinyl ketone are dissolved in 250 grams of dioxan and agitated overnight with 50 grams of cyclohexylamine. A test showed that the resin was not readily soluble in dilute acids; hence, the reaction mixture is heated in a steam bath for 5 hours. The resin is then precipitated. By pouring the reaction mixture in water and after standing 12 hours in fresh water, it is filtered and dried in vacuo. The yield is 55 grams. The pulverized resin is soluble to the extent of 4 grams in 96 grams of 5% aqueous solution of acetic acid.

*Example E*

A solution of 18 grams (0.4 mol.) of dimethylamine in 32.4 grams (0.4 mol.) of 37% aqueous formaldehyde was added with mechanical stirring and cooling to 53.5 grams (0.5 mol.) of 88% phenol. To the above mixture, a solution of 81 grams (1 mol.) of 37% aqueous formaldehyde and 30.4 grams (0.5 mol.) of 28% aqueous ammonia was added with cooling. The resulting solution was gradually heated in a water bath to 90° C. and held at that temperature for 5 hours. The resulting resin was purified by grinding it to a uniform slurry in the presence of a little water in an ice cold mortar, followed by filtration and washing with ice cold water. After drying, it weighed 74 grams. It was a yellow material which softened slightly above room temperature. It was soluble in acetone, ethyl acetate, dioxan, 10% aqueous sodium hydroxide, 1.5% aqueous acetic acid, 3% formic acid, and 90% toluene-10% ethanol mixture.

There are of course numerous other amino polymers that can be prepared in much the same way as will be apparent from a study of the ap-

plications specifically referred to above, such as for instance beta-dimethylaminomethyl methacrylate; beta-dicyclohexylaminomethyl methacrylate; beta-di-N-butylaminomethyl methacrylate; betamorpholine-N-ethyl methacrylate; triethanolamine monomethacrylate; dimethylaminomethyl zein; diethylaminomethyl zein; dibutylaminomethyl zein; piperidyl methyl glycine; dimethylaminomethyl gladin; dimethylaminomethyl casein; the polymerization product resulting by reacting polymeric methyl vinyl ketone with concentrated ammonium hydroxide or with amines such as cyclohexylamine, glucamine, ethanolamine, ethylene diamine; the reaction product between phenol, formaldehyde, ammonia and dimethylamine; between phenol, lignin, formaldehyde and dimethylamine; between phenol, formaldehyde and dimethylaminomethanol; between phenol, formaldehyde and dimethylol cyclohexanolamine; between phenol, formaldehyde, ammonia and aniline; and many others.

Instead of simple polymers, interpolymers may be prepared, for instance by reacting methyl methacrylate and methyl vinyl ketone in the presence of ammonium hydroxide or reacting beta-cyclohexylaminomethyl methacrylate monomer and beta-dimethylaminomethyl methacrylate monomer together under suitable conditions. Other equivalent polymeric materials such as copolymers may also be used, provided their solubility characteristics are as previously set forth.

In order that the finished cellulosic sheet may be of the desired degree of softness, a softening agent, such as glycerin, is incorporated in the aqueous solution of the size. The aqueous solution may be applied to the cellulosic sheet by immersing the sheet in the solution or by brushing or spraying the solution onto the sheet, or by applying the solution to the sheet by rollers or by any other convenient means. Moreover, the size solution may be applied either to the cellulosic sheet in the gel condition or to the finished dry cellulosic sheet by another operation. We prefer, however, to apply it to the gel sheet from the glycerin bath. In the step of drying the cellulosic sheet treated with a solution of the size, for example, the acetate of de-acetylated chitin, in which step the soluble salt is converted to an insoluble coating or sizing on the sheet, a wide range of temperature is possible. We prefer, however, to carry out the drying operation at temperatures between 50 degrees and 90 degrees centigrade. In certain cases, as has been stated in the preceding paragraph, vapors of basic compounds, such as ammonia, may be caused to act on the cellulosic sheet during the drying operation or on the cellulosic sheet after drying if it is desired to facilitate the conversion of the size salt to an insoluble product. The same effect may be achieved by treating the cellulosic sheet, which has been dried or partially dried after the application of the solution of the size, with a solution of a basic compound, such as dilute ammonium hydroxide, a solution of ethylene diamine, or of triethanolamine or the like.

As has been stated, the greatest advantages follow from the use of de-acetylated chitin as an anchoring agent for moistureproofing coatings applied to regenerated cellulose or to other cellulosic films of the character described. It will be understood that it can in general be used to anchor coatings for transparent cellulosic sheeting where such coatings have less or greater moistureproofing properties than those described in the examples given above.

The present invention effects the production of flexible, substantially odorless, non-fibrous, non-porous cellulosic sheets or films having a moistureproofing coating securely anchored to the film base and resistant to deterioration when subjected to the action of liquid water over long periods of time. Further advantages are the adaptability of the process of the invention to equipment now used for the production of regenerated cellulose film and the like, without necessitating a substantial change in the design of such equipment; lower cost, minimum waste and great efficiency. Where no pigment is used, the composite films have a high degree of transparency.

The term "de-acetylated chitin", as used in the claims, is intended to include the product which is prepared by removing the acetyl groups from chitin in any suitable way. Unless otherwise qualified, the term also includes the product prepared by solubilizing the de-acetylated chitin, as, for example, by forming a salt with an acid, and by again insolubilizing. It is also intended to include any other product substantially identical therewith, as, for example, where such product is produced synthetically.

In some instances the dried cellulosic sheet coated or sized with de-acetylated chitin may retain a very faint trace of the characteristic odor of the acid used in forming the water-soluble salt. This trace of odor may readily be removed by treating the sheet with dilute vapors or a dilute solution of a basic compound like ammonia to neutralize the acid, by volatilizing the acid by means of heat, or by a current of air or steam, or by any known deodorizing treatment. If desired, the aqueous solution of the size may be subjected to treatment with activated carbon in order to remove any undesirable odor.

While the invention has been described particularly with respect to transparent wrapping tissues, it will be understood that within its broad scope, the invention includes the anchoring of coatings to sheets which are thicker than wrapping tissues. The invention is also applicable to the anchoring of coatings to tubes, sausage casings, bottle caps and bands, molded articles, and, in general, to any articles of cellulose or similar material of the character described, where the problem of anchoring coatings arises.

The preferred form of the invention resides in the anchoring of moistureproofing surface coatings to a non-porous, non-fibrous base such as regenerated cellulose. Within its broadest scope, the invention comprehends also the coating of other bases, e. g., rayon fabric and the like, in order to anchor surface coatings thereto. Even where the coating of the base, whether it be non-porous or of other character, is discontinuous in character, such, for example, as in the printing of colors, symbols, indicia, advertisements, etc., the de-acetylated chitin may be used as the anchoring agent. Thus, regenerated cellulose sheets, tubes, caps, sausage casing, etc., when coated or sized with de-acetylated chitin may be printed with printing ink either having a lacquer base or a drying-oil base, to give any desired indicia, and, after drying, the printing remains securely anchored to the base even after being subjected to rigid washing, boiling or other processing steps.

Additionally, the present invention may be used to improve the anchorage of various coatings to bases other than those specifically noted above, for example, paper, cotton cloth, and

other bases which are water sensitive, i. e., will absorb water, the anchoring agents improving the adhesion between the coating and base over that exhibited where the coating is applied to the base in the absence of the anchoring agent.

The invention also contemplates the production of coated self-sustaining films of de-acetylated chitin formed by casting or otherwise forming the de-acetylated chitin into the desired form and then applying a coating.

For the purposes of this invention, moisture-proof materials are defined as those which, in the form of a thin, continuous and unbroken film, will permit the passage of not more than 690 grams of water vapor per 100 square meters per hour, over a period of 24 hours at approximately 39.5° C.  $\pm 0.5$ ° C., the relative humidity of the atmosphere at one side of the film being maintained at least at 98% and the relative humidity of the atmosphere at the other side being maintained at such value as to give a humidity differential of at least 95%.

Moistureproofing coating compositions are defined as those which, when laid down in the form of thin, continuous, unbroken films, applied uniformly as a coating with a total thickness not exceeding 0.0005" to both sides of a sheet of regenerated cellulose of thickness approximately 0.0009", will produce a coated product which is moistureproof.

A moistureproofed regenerated cellulose sheet is capable of resisting the passage of moisture or water vapor at least ten times as effectively as the uncoated regenerated cellulose sheet.

Parts, proportions and/or percentages referred to throughout the specification and claims are to be construed as parts, proportions and/or percentages by weight unless indicated otherwise.

Any variation of or modification of the invention, as it has been described above in this application, which conforms to the spirit of the invention, is intended to be included within the scope of the claims.

We claim:

1. An article of manufacture comprising a water-sensitive base, a surface coating and an intermediate coating comprising an amino polymer which is substantially insoluble in water and in 5% aqueous ammonia but soluble in 2% aqueous acetic acid.

2. An article of manufacture comprising a water-sensitive non-fibrous base, a surface coating and an intermediate coating comprising an amino polymer which is substantially insoluble in water and in 5% aqueous ammonia but soluble in 2% aqueous acetic acid.

3. A composite film suitable for use as a wrapping tissue comprising a water-sensitive, non-fibrous base, a surface coating and an intermediate coating comprising an amino polymer which is substantially insoluble in water and in 5% aqueous ammonia but soluble in 2% aqueous acetic acid.

4. A composite film suitable for use as a wrapping tissue comprising a water-sensitive, non-fibrous base, a moistureproofing coating and an intermediate coating comprising an amino polymer which is substantially insoluble in water and in 5% aqueous ammonia but soluble in 2% aqueous acetic acid.

5. In a process for producing an article comprising a water-sensitive base and a surface coating which adheres tenaciously to the base even when in contact with water over long periods of time, the steps which comprise applying to the

- base an intermediate coating comprising an amino polymer which is substantially insoluble in water and in 5% aqueous ammonia but soluble in 2% aqueous acetic acid, then applying a surface coating.
6. In a process for producing an article comprising a water-sensitive, non-fibrous base and a surface coating which adheres tenaciously to the base even when in contact with water over long periods of time, the steps which comprise applying to the base an intermediate coating comprising an amino polymer which is substantially insoluble in water and in 5% aqueous ammonia but soluble in 2% aqueous acetic acid, then applying a surface coating.
7. A composite film suitable for use as a wrapping tissue comprising a non-fibrous cellulosic sheet, an intermediate coating comprising a de-acetylated chitin, and a surface coating, said sheet and said surface coating exhibiting an adhesion greatly improved over that exhibited between a similar sheet and surface coating when in direct contact with each other, said adhesion being tenacious even when the composite film is subjected to contact with water over a long period of time.
8. A composite film suitable for use as a wrapping tissue comprising a sheet of regenerated cellulose, an intermediate coating comprising a de-acetylated chitin, and a surface coating.
9. A composite film suitable for use as a wrapping tissue comprising a sheet of regenerated cellulose, an intermediate coating comprising a de-acetylated chitin, and a surface coating comprising a moistureproofing composition.
10. A composite film suitable for use as a wrapping tissue comprising a non-fibrous cellulosic sheet, an intermediate coating of a de-acetylated chitin, and a surface coating which contains a cellulose derivative base, said sheet and said surface coating exhibiting an adhesion greatly improved over that exhibited between a similar sheet and surface coating when in direct contact with each other, said adhesion being tenacious even when the composite film is subjected to contact with water over a long period of time.
11. In a process for preparing a product suitable for use as a wrapping tissue, the steps comprising applying an aqueous solution of a solubilized de-acetylated chitin to a sheet of regenerated cellulose, drying the treated sheet, and then applying a moistureproofing surface coating.
12. A composite film suitable for use as a wrapping tissue comprising a sheet of regenerated cellulose, an intermediate coating of a member of the class consisting of de-acetylated chitin and de-acetylated chondroitin and a surface coating.
13. A printed article comprising a water sensitive base having printing thereon and provided with an anchoring agent for the printing comprising a de-acetylated chitin.
14. A moistureproof composite film suitable for use as a wrapping tissue comprising a sheet of regenerated cellulose, an intermediate coating of a de-acetylated chitin, and a surface coating comprising a moistureproofing cellulose derivative composition.
15. In a process of producing a product suitable for use as a wrapping tissue and comprising a base and surface coating which exhibit a greatly improved adhesion of such a character as to remain tenacious when subjected to contact with water over long periods of time, the steps which comprise applying a coating comprising a solution of de-acetylated chitin to a non-fibrous, cellulosic sheet, drying the sheet, and then applying a surface coating.
16. The process of claim 15 characterized in that the solution is an aqueous solution of a salt of a de-acetylated chitin and an acid.
17. The process of claim 15 characterized in that the solution is an aqueous solution of a salt of a de-acetylated chitin and an acid, said solution also containing a softener for the cellulosic sheet.
18. The process of claim 15 characterized in that the solution is an aqueous solution of a salt of a de-acetylated chitin and an acid, and further characterized in that the sheet is treated with a basic material prior to applying the surface coating.
19. The process of claim 15 characterized in that the solution is an aqueous solution of a salt of a de-acetylated chitin and an acid, and further characterized in that the sheet is treated with gaseous ammonia during drying.
20. A composite article comprising a water-sensitive base, an intermediate coating of the class consisting of de-acetylated chitin and de-acetylated chondroitin, and a surface coating, said base and said surface coating exhibiting an adhesion greatly improved over that exhibited between a similar base and surface coating when in direct contact with each other, said adhesion being tenacious even when the composite film is subjected to contact with water over long periods of time.
21. The process which comprises applying a fluid coating composition to de-acetylated chitin, converting the coating composition into a solid coating, whereby to obtain a composite article in which the coating adheres to the de-acetylated chitin tenaciously even when the composite article is subjected to the action of water for a long period of time.
22. A composite article comprising a water-sensitive cellulosic base, a surface coating thereon and an intermediate coating of de-acetylated chitin, the coating being anchored tenaciously to the base even when the composite article is subjected for a long period of time to the action of water, the coating and base exhibiting an adhesion greatly improved over that exhibited between a similar coating and base when in direct contact with each other.

ERNEST K. GLADDING.  
DOROTHY BATEMAN MANEY.